

# UNITED STATES PATENT OFFICE.

WILHELM SCHUMACHER, OF BERLIN, GERMANY, ASSIGNOR TO GENERAL BRIQUETTING COMPANY, OF NEW YORK, N. Y., A CORPORATION OF MAINE.

## AGGLOMERATION OF FINE ORES AND FLUE-DUST.

1,222,893.

Specification of Letters Patent. Patented Apr. 17, 1917.

No Drawing.

Application filed January 26, 1916. Serial No. 74,518.

To all whom it may concern:

Be it known that I, WILHELM SCHUMACHER, a citizen of the German Empire, and a resident of Berlin, Germany, have invented certain new and useful Improvements in and Relating to the Agglomeration of Fine Ores and Flue-Dust, of which the following is a specification.

My invention relates to the agglomeration, particularly the sintering and roasting of fine ores, concentrates, flue dust and the like and has for its object the accomplishment of such agglomeration using the said ores in the form of small, ball-like briquets, and employing ordinary furnaces, such as shaft furnaces. This and other objects as will hereinafter appear are attained in the following manner.

The fine ore or equivalent material is first molded into small briquets having substantially the form of regular solids the surfaces of which are curved; for example, the briquets may be spherical or egg-shaped. These ball-like briquets are now carefully introduced either continuously or intermittently into a suitable furnace such as a shaft furnace or kiln and subjected to a suitable temperature to accomplish roasting or agglomeration. The special advantage of employing briquets of the shape indicated is due to the fact that each briquet touches its neighbors with contact areas of small dimensions approaching the area of a point. In other words the contacts between the briquets may be said to be point contacts rather than surface contacts. Thus the spaces between the briquets are uniform cavities connected with each other, and serve as a system of tubes of geometrical uniformity. The combustion air and the gases, such as the gaseous products of combustion, can therefore pass unhindered through all of these channels of comparatively large cross-section, and fully bathe, so to speak, all the briquets, thereby heating them all to the same temperature. The briquets are homogeneously distributed and the gas passages between them are homogeneous in structure so that the gases will readily pass through all of the passages in uniform flow and will not find, as often happens with such furnaces in which fine or irregularly shaped material is being treated, preferred channels or flues through which the bulk of the gases escapes, thus heating the material in the neighborhood of such

flues to a temperature higher than necessary and failing to heat the other material to a sufficiently high temperature.

The briquets of the present invention, moreover, are of small diameter, say the size of a hen's egg; the temperature difference between the superficial portions and the interior portions of the briquet is therefore negligibly low so that the action is not the same as with large pieces in which case rapid heating causes the outer portions to melt while the inner cores have a temperature lower than that required to sinter the material. For this reason and on account of the facility with which the combustion gases are allowed to pass in contact with all of the briquets, the treatment, in accordance with my process, requires both less time and less fuel.

Agglomeration, by which I include sintering and roasting, of fine ores and the like is particularly difficult as the sintering point and the melting point are relatively close together, for which reason it sometimes happens with processes used heretofore that the sintering temperature is not reached and a sintering of the material is not effected, at least not homogeneously effected, while on the other hand the melting temperature is exceeded and the material, or a part of it, is melted. In either case the purpose of agglomeration, that is the utilization of the fine ores, is not effected or is only partially effected.

If briquets with large plane surfaces such as rectangular briquets, in contradistinction to the ball-like briquets of my invention, are used, as in the past, for the roasting process, large piles are produced and at the same time irregular hole-like spaces are created. The result is that the material is not uniformly heated and in such a case the product will not be uniform.

The simplest and cheapest way in which my briquets may be formed is perhaps by means of egg briquetting presses such as are used in the coal briquetting industry and in some instances have been used for the briquetting of ore with sulfite pitch as a binder; these briquets, however, are charged directly into blast furnaces and do not undergo a roasting operation. Briquets which are to be agglomerated, on the other hand, need not necessarily contain a binder, the ores themselves being somewhat plastic, while

only a small percentage of binder can be added to briquets for blast furnace use.

The egg briquets can be either roasted with gas or coal by properly apportioning the latter between the briquets or briquetting the coal together with the fine ores. This last method offers special advantages as the coal is spread throughout the mass with absolute uniformity; consequently the temperature is the same throughout the zone of combustion and the product obtained is exceptionally uniform.

Egg briquets can be used for any roasting apparatus that has been used in the past for fine ores in pulverized or lump form. The shaft furnace, however, offers special advantages in this instance as it always has been utilized in the past for sintering fine ores that were not in lump form. The roasting operation can almost wholly be accomplished automatically by feeding the briquets directly from the press into the top of the furnace by means of a conveyer belt while at the bottom a rotating disk can be installed with a device for discharging the briquets automatically. As the roasting operation goes on rapidly, the furnace contents are kept in continual movement which prevents the briquets from clinging to one another in the sintering or roasting zone. This beneficial result is greatly aided by the form or shape which I give to my briquets because of the fact that the contact surfaces of the adjacent briquets are reduced to a minimum and that, therefore, the minimum fusion of the adjacent briquets to each other takes place. The briquets will, therefore, when agitated, remain separated units and when sintering takes place without agitation a separation may be effected after the com-

pletion of the processes with a minimum amount of difficulty. It is obvious that in order to be adapted for the treatment in a shaft furnace as described, the structure of the briquets must be what I call of a permanent character as distinguished from a briquet which has been merely shaped but is not strong enough to withstand handling.

When in my claims I speak of fine ores I mean, of course, to include flue dust and other metal bearing substances which are in a finely divided state and which have the characteristic, hereinabove mentioned, of having their sintering and melting points relatively close together.

I claim:

1. That improvement in the art of agglomerating fine ores which consists in incorporating in the form of small, permanent, ball-like or egg-shaped briquets the finely divided particles of such fine ores whose sintering and melting points are relatively close together and then exposing such briquets to a temperature between the sintering and melting temperature of the ores.

2. That improvement in the art of agglomerating fine ores which consists in incorporating in the form of small, permanent, ball-like or egg-shaped briquets the finely divided particles of such fine ores whose sintering and melting points are relatively close together, then exposing such briquets to a temperature between the sintering and melting temperature of the ores and maintaining continual movement of the briquets while in the sintering or roasting zone.

In testimony whereof I have hereunto set my hand.

WILHELM SCHUMACHER.